



US010351921B2

(12) **United States Patent**  
**Snyder et al.**

(10) **Patent No.:** **US 10,351,921 B2**  
(b5) **Date of Patent:** **Jul. 16, 2019**

(54) **MARTENSITIC STAINLESS STEEL STRENGTHENED BY COPPER-NUCLEATED NITRIDE PRECIPITATES**

(71) Applicant: **QuesTek Innovations LLC**

(72) Inventors: **David R. Snyder**, Des Plaines, IL (US); **Jiadong Gong**, Evanston, IL (US); **Jason T. Sebastian**, Chicago, IL (US); **James A. Wright**, Los Gatos, CA (US); **Herng-Jeng Jou**, San Jose, CA (US); **Zechariah Feinberg**, Mountain View, CA (US)

(73) Assignee: **QuesTek Innovations LLC**, Evanston, IL (US)

(\*) Notice: Subject to any disclaimer, the term of this patent is extended or adjusted under 35 U.S.C. 154(b) by 53 days.

(21) Appl. No.: **15/819,472**

(22) Filed: **Nov. 21, 2017**

(65) **Prior Publication Data**

US 2018/0135143 A1 May 17, 2018

**Related U.S. Application Data**

(60) Continuation of application No. 14/462,119, filed on Aug. 18, 2014, now abandoned, which is a division of  
(Continued)

(51) **Int. Cl.**  
**C22C 38/00** (2006.01)  
**C21D 6/02** (2006.01)  
(Continued)

(52) **U.S. Cl.**  
CPC ..... **C21D 6/02** (2013.01); **C21D 6/004** (2013.01); **C21D 6/005** (2013.01); **C21D 6/007** (2013.01);  
(Continued)

(58) **Field of Classification Search**

CPC ..... C21D 6/02; C21D 6/005; C21D 6/004;  
C21D 6/007; C22C 38/04; C22C 38/52;  
(Continued)

(56) **References Cited**

U.S. PATENT DOCUMENTS

2,797,993 A 7/1957 Tanczyn  
2,926,111 A 2/1960 Schweitzer

(Continued)

FOREIGN PATENT DOCUMENTS

DE 2453109 A1 5/1975  
EP 0386673 A1 9/1990

(Continued)

OTHER PUBLICATIONS

Mar. 5, 2018—U.S. Final Office Action—U.S. Appl. No. 14/691,956.  
(Continued)

*Primary Examiner* — Kiley S Stoner

(74) *Attorney, Agent, or Firm* — Banner & Witcoff, Ltd.

(57) **ABSTRACT**

A martensitic stainless steel alloy is strengthened by copper-nucleated nitride precipitates. The alloy includes, in combination by weight percent, about 10.0 to about 12.5 Cr, about 2.0 to about 7.5 Ni, up to about 17.0 Co, about 0.6 to about 1.5 Mo, about 0.5 to about 2.3 Cu, up to about 0.6 Mn, up to about 0.4 Si, about 0.05 to about 0.15 V, up to about 0.10 N, up to about 0.035 C, up to about 0.01 W, and the balance Fe and incidental elements and impurities. The nitride precipitates may be enriched by one or more transition metals. A case hardened, corrosion resistant variant has a reduced weight percent of Ni, enabling increased use of Cr, and decreased Co.

**8 Claims, 5 Drawing Sheets**



**Related U.S. Application Data**

application No. 12/937,348, filed as application No. PCT/US2009/040351 on Apr. 13, 2009, now Pat. No. 8,808,471, application No. 15/819,472, which is a continuation of application No. 14/574,611, filed on Dec. 18, 2014, now Pat. No. 9,914,987.

(60) Provisional application No. 61/044,355, filed on Apr. 11, 2008.

**(51) Int. Cl.**

**C22C 38/20** (2006.01)  
**C22C 38/42** (2006.01)  
**C22C 38/44** (2006.01)  
**C22C 38/46** (2006.01)  
**C21D 6/00** (2006.01)  
**C22C 38/02** (2006.01)  
**C22C 38/52** (2006.01)  
**C22C 38/04** (2006.01)

**(52) U.S. Cl.**

CPC ..... **C22C 38/01** (2013.01); **C22C 38/02** (2013.01); **C22C 38/04** (2013.01); **C22C 38/20** (2013.01); **C22C 38/42** (2013.01); **C22C 38/44** (2013.01); **C22C 38/46** (2013.01); **C22C 38/52** (2013.01)

**(58) Field of Classification Search**

CPC ..... C22C 38/02; C22C 38/001; C22C 38/20; C22C 38/42; C22C 38/44; C22C 38/46

USPC ..... 420/8-129

See application file for complete search history.

**(56)****References Cited****U.S. PATENT DOCUMENTS**

4,154,629 A 5/1979 Asai et al.  
 4,420,335 A 12/1983 Takagi et al.  
 4,434,006 A 2/1984 Kato et al.  
 4,659,241 A 4/1987 Bamberger et al.  
 5,089,067 A 2/1992 Schumacher  
 5,310,431 A 5/1994 Buck  
 5,545,269 A 8/1996 Koo et al.  
 5,650,024 A 7/1997 Hasegawa et al.  
 5,785,924 A 7/1998 Beguinot et al.  
 5,900,075 A 5/1999 Koo et al.  
 6,045,633 A 4/2000 Henn et al.  
 6,162,389 A 12/2000 Hase et al.  
 6,228,183 B1 5/2001 Bangaru et al.  
 6,245,290 B1 6/2001 Koo et al.  
 6,248,191 B1 6/2001 Luton et al.  
 6,264,760 B1 7/2001 Tamehiro et al.  
 6,764,647 B2 7/2004 Aigner et al.  
 6,793,744 B1 9/2004 Jung  
 7,070,663 B2 7/2006 Suzuki et al.  
 7,160,399 B2 1/2007 Kuehmann et al.  
 7,186,304 B2 3/2007 Chin et al.  
 7,235,212 B2 6/2007 Kuehmann et al.  
 7,887,645 B1 2/2011 Schoen et al.  
 8,715,432 B2 5/2014 Hasegawa et al.  
 2002/0139449 A1 10/2002 Goecmen  
 2002/0164260 A1 11/2002 Koga et al.  
 2003/0102057 A1 6/2003 Short  
 2003/0192626 A1 10/2003 Takiguchi et al.  
 2004/0096351 A1 5/2004 Suzuki et al.

|                  |         |                                           |
|------------------|---------|-------------------------------------------|
| 2004/0191109 A1  | 9/2004  | Maziasz et al.                            |
| 2006/0021682 A1* | 2/2006  | Saha ..... C21D 1/20<br>148/547           |
| 2006/0060270 A1  | 3/2006  | Clueh et al.                              |
| 2006/0096671 A1  | 5/2006  | Sano et al.                               |
| 2006/0163231 A1* | 7/2006  | Kobayashi ..... B23K 35/308<br>219/146.23 |
| 2007/0000576 A1  | 1/2007  | Blanke                                    |
| 2008/0138233 A1  | 6/2008  | Tomita et al.                             |
| 2008/0251166 A1  | 10/2008 | Han                                       |
| 2009/0194175 A1  | 8/2009  | Gerceker et al.                           |
| 2009/0277539 A1  | 11/2009 | Kimura et al.                             |
| 2009/0291014 A1  | 11/2009 | Vartanov                                  |
| 2009/0324441 A1  | 12/2009 | Weiss et al.                              |
| 2011/0024003 A1  | 2/2011  | Vartanov                                  |
| 2012/0031529 A1  | 2/2012  | Ohishi et al.                             |
| 2016/0040262 A1  | 2/2016  | Snyder et al.                             |

**FOREIGN PATENT DOCUMENTS**

|    |                     |         |
|----|---------------------|---------|
| EP | 0607263 B1          | 12/1999 |
| EP | 1158065 A1          | 11/2001 |
| EP | 1602744 B1          | 3/2009  |
| FR | 2700174 A1          | 7/1994  |
| GB | 678616 A            | 9/1952  |
| GB | 2179675 A           | 3/1987  |
| JP | WO 2008/016158 A1 * | 2/2008  |
| WO | 9102827 A1          | 3/1991  |
| WO | 9840180 A1          | 9/1998  |
| WO | 03018856 A2         | 3/2003  |
| WO | 2005014873 A1       | 2/2005  |
| WO | 2006068610 A1       | 6/2006  |
| WO | 2006081401 A2       | 8/2006  |
| WO | 2008123159 A1       | 10/2008 |
| WO | 2009126954 A2       | 10/2009 |
| WO | 2010149561 A1       | 12/2010 |

**OTHER PUBLICATIONS**

Oct. 9, 2018—U.S. Non Final OA—U.S. Appl. No. 14/691,956.  
 Oct. 21, 2010—(PCT) International Preliminary Report—PCT/US2009/040351.  
 Mar. 18, 2010—(PCT)—International Search Report and Written Opinion—PCT/US2009/040351.  
 Ageev V S; Vil'Danova N F; Kozlov K A; Kochetkova T N; Nikitina A A; Sagardzze V V; Safronov B V; Tsvelev V V; Chukanov A P: "Structure and thermal creep of the oxide-dispersion-strengthened EP-450 reactor steel" Physics of Metals and Metallography Sep. 2008—Maik Nauka-Interperiodica Publishing, vol. 106, No. 3, Sep. 2008 (Sep. 2008), pp. 318-325, XP002571196 RU ISSN: 0031-918X DOI: 10.1134/S0031918X08090123.  
 Frandsen R B et al: "Simultaneous surface engineering and bulk hardening of precipitation hardening stainless steel" Surface and Coatings Technology, Elsevier, Amsterdam, NL, vol. 200, No. 16-17, Apr. 27, 2006 (Apr. 27, 2006), pp. 5160-5169, XP024995358 ISSN: 0257-8972 DOI: 10.1016/j.surcoat.2005.04.038 [retrieved on Apr. 27, 2006].  
 Feb. 8, 2016—(PCT)—International Search Report and Written Opinion—App PCT/US2015/027073.  
 Mar. 3, 2018—U.S. Final Office Action—U.S. Appl. No. 14/691,956.  
 Jul. 6, 2017—U.S. Non-Final Office Action—U.S. Appl. No. 14/691,956.  
 Jun. 21, 2017—U.S. Non-Final Office Action—U.S. Appl. No. 14/462,119.  
 Jun. 22, 2017—U.S. Non-Final Office Action U.S. Appl. No. 14/574,611.

\* cited by examiner



FIG. 1



FIG. 2

## N63-2X Data/properties



FIG. 3

FIG. 4

## N63-2X Data/properties - B117 Salt Fog Testing



FIG. 5



FIGURE 6

## 1

**MARTENSITIC STAINLESS STEEL  
STRENGTHENED BY COPPER-NUCLEATED  
NITRIDE PRECIPITATES**

**CROSS-REFERENCE TO RELATED  
APPLICATIONS**

This is a continuation application of U.S. Ser. No. 14/574,611 filed Dec. 18, 2014 and U.S. Ser. No. 14/462,119 filed Aug. 18, 2014 which claims priority to and the benefit of U.S. Provisional Patent Application No. 61/044,355, filed Apr. 11, 2008, PCT Application Number PCT/US2009/040351 filed Apr. 13, 2009 and U.S. Utility patent application Ser. No. 12/937,348 filed Nov. 29, 2010 which is incorporated by reference herein and made part hereof.

**FEDERALLY SPONSORED RESEARCH AND  
DEVELOPMENT**

This invention may be subject to governmental license rights pursuant to Marine Corps Systems Command Contract No. M67854-05-C-0025, Navy Contract No. N68335-12-C-0248 and Navy Contract No. N68335-13-0280.

**BACKGROUND**

The material properties of secondary-hardened carbon stainless steels are often limited by cementite precipitation during aging. Because the cementite is enriched with alloying elements, it becomes more difficult to fully dissolve the cementite as the alloying content of elements such as chromium increases. Undissolved cementite in the steel can limit toughness, reduce strength by gettering carbon, and act as corrosion pitting sites.

Cementite precipitation could be substantially suppressed in stainless steels by substituting nitrogen for carbon. There are generally two ways of using nitrogen in stainless steels for strengthening: (1) solution-strengthening followed by cold work; or (2) precipitation strengthening. Cold worked alloys are not generally available in heavy cross-sections and are also not suitable for components requiring intricate machining. Therefore, precipitation strengthening is often preferred to cold work. Precipitation strengthening is typically most effective when two criteria are met: (1) a large solubility temperature gradient in order to precipitate significant phase fraction during lower-temperature aging after a higher-temperature solution treatment, and (2) a fine-scale dispersion achieved by precipitates with lattice coherency to the matrix.

These two criteria are difficult to meet in conventional nitride-strengthened martensitic steels. The solubility of nitrogen is very low in the high-temperature bcc-ferrite matrix. And in austenitic steels, nitrides such as  $M_2N$  are not coherent with the fcc matrix. Thus, there has developed a need for a martensitic steel strengthened by nitride precipitates.

Ideally, such steels will be corrosion resistant and exhibit high case hardness accompanied by excellent core properties including tensile yield strength above 150 ksi, tensile ultimate strength above 190 ksi, high fracture toughness and good elongation properties.

**BRIEF SUMMARY**

Aspects of the present invention relate to a martensitic stainless steel strengthened by copper-nucleated nitride precipitates. According to some aspects, the steel substantially

## 2

excludes cementite precipitation during aging. Cementite precipitation can significantly limit strength and toughness in the alloy.

According to other aspects, the steel of the present invention is suitable for casting techniques such as sand casting, because the solidification range is decreased, nitrogen bubbling can be substantially avoided during the solidification, and hot shortness can also be substantially avoided. For some applications, the steel can be produced using conventional low-pressure vacuum processing techniques known to persons skilled in the art. The steel can also be produced by processes such as high-temperature nitriding, powder metallurgy possibly employing hot isostatic pressing, and pressurized electro slag remelting.

According to another aspect, a martensitic stainless steel includes, in combination by weight percent, about 10.0 to about 12.5 Cr, about 2.0 to about 7.5 Ni, up to about 17.0 Co, about 0.6 to about 1.5 Mo, about 0.5 to about 2.3 Cu, up to about 0.6 Mn, up to about 0.4 Si, about 0.05 to about 0.15 V, up to about 0.10 N, up to about 0.035 C, up to about 0.01 W, and the balance Fe.

According to another aspect, a martensitic stainless steel includes, in combination by weight percent, about 10.0 to about 14.5 Cr, about 0.3 to about 7.5 Ni, up to about 17.0 Co, about 0.6 to about 1.5 Mo, about 0.25 to about 2.3 Cu, up to about 0.6 Mn, up to about 0.4 Si, about 0.05 to about 0.15 V, up to about 0.10 N, Carbon up to about 0.2 C, up to about 0.01 W, and the balance Fe and wherein the alloy is case hardened with a primarily martensitic microstructure preferably in the range of at least about 90% by volume.

Another aspect of the invention is to provide a martensitic stainless steel embodiment which is corrosion resistant, which may be case hardened with a primarily martensitic case layer strengthened by copper-nucleated nitride precipitates.

**BRIEF DESCRIPTION OF THE DRAWINGS**

FIG. 1 is a graph illustrating the Rockwell C-scale hardness of an embodiment of an alloy according to the present invention, at specified aging conditions;

FIG. 2 is a three-dimensional computer reconstruction of a microstructure of an embodiment of an alloy according to the present invention, produced using atom-probe tomography;

FIG. 3 is a graph depicting the case hardness of five separate examples of a variant alloy of the invention;

FIG. 4 is a graph depicting the quantity of retained austenite in the case of the five reported variant experimental alloys identified in Tables 2 and 3 which in turn identify the experimental and measured chemistry analysis in weight percent of the five experimental alloys illustrating the invention;

FIG. 5 is a photograph depicting the visual result of a corrosion test performed on two of the alloys of the invention in comparison to first and second control specimens; and

FIG. 6 is a flow diagram or graphical representation of the method or processing of the disclosed alloy to achieve core and case properties.

**DETAILED DESCRIPTION**

In one embodiment, a steel alloy includes, in combination by weight percent, about 10.0 to about 14.5 Cr, about 2.0 to about 7.5 Ni, up to about 17.0 Co, about 0.6 to about 1.5 Mo, about 0.25 to about 2.3 Cu, up to about 0.6 Mn, up to about

0.4 Si, about 0.05 to about 0.15 V, up to about 0.10 N, up to about 0.2 C, up to about 0.01 W, and the balance Fe and incidental elements and impurities. In another embodiment, the alloy includes, in combination by weight percent, about 10.0 to about 12.0 Cr, about 6.5 to about 7.5 Ni, up to about 4.0 Co, about 0.7 to about 1.3 Mo, about 0.5 to about 1.0 Cu, about 0.2 to about 0.6 Mn, about 0.1 to about 0.4 Si, about 0.05 to about 0.15 V, up to about 0.09 N, about 0.005 to about 0.035 C, and the balance Fe and incidental elements and impurities. In this embodiment, the content of cobalt is minimized below 4 wt % and an economic sand-casting process is employed, wherein the steel casting is poured in a sand mold, which can reduce the cost of producing the steel. It is understood that a greater amount of cobalt can be used in this embodiment. For example, secondary-hardened carbon stainless steels disclosed in U.S. Pat. Nos. 7,160,399 and 7,235,212, which are incorporated by reference herein and made part hereof, have a cobalt content up to about 17 weight percent. To establish a nitride-strengthened analogue of carbide-strengthened stainless steels, a cobalt content of up to about 17 weight percent may be utilized in this embodiment.

To be suitable for sand-casting, the solidification temperature range is minimized in this embodiment. During this solidification, nitrogen bubbling can be avoided by deliberately choosing the amount of alloying additions, such as chromium and manganese, to ensure a high solubility of nitrogen in the austenite. The very low solubility of nitrogen in bcc-ferrite phase can present an obstacle to the production of nitride-strengthened martensitic stainless steels. To overcome this challenge, one embodiment of the disclosed steel solidifies into fcc-austenite instead of bcc-ferrite, and further increases the solubility of nitrogen with the addition of chromium. The solidification temperature range and the desirable amount of chromium can be computed with thermodynamic database and calculation packages such as Thermo-Calc® software and the kinetic software DIC-TRATM (Diffusion Controlled TRAnsformations) version 24 offered by Thermo-Calc Software. In another embodiment, the cast steel subsequently undergoes a hot isostatic pressing at 1204° C. and 15 ksi Ar for 4 hours to minimize porosity.

Compared to conventional nitride-strengthened steels, embodiments of the disclosed steel alloy have substantially increased strength and avoided embrittlement under impact loading. In one embodiment, the steel exhibits a tensile yield strength of about 1040 to 1360 MPa, an ultimate tensile strength of about 1210 to 1580 MPa, and an ambient impact toughness of at least about 10 ft-lb. In another embodiment, the steel exhibits an ultimate tensile strength of 1240 MPa (180 ksi) with an ambient impact toughness of 19 ft-lb. Upon quenching from a solution heat treatment, the steel transforms into a principally lath martensitic matrix. To this end, the martensite start temperature ( $M_s$ ) is designed to be at least about 50° C. in one embodiment, and at least about 150° C. in another embodiment. During subsequent aging, a

copper-based phase precipitates coherently. Nanoscale nitride precipitates enriched with transition metals such as chromium, molybdenum, and vanadium, then nucleate on these copper-based precipitates. In one embodiment, these nitride precipitates have a structure of  $M_2N$ , where M is a transition metal. Additionally, in this embodiment, the nitride precipitates have a hexagonal structure with two-dimensional coherency with the martensite matrix in the plane of the hexagonal structure. The hexagonal structure is not coherent with the martensite matrix in the direction normal to the hexagonal plane, which causes the nitride precipitates to grow in an elongated manner normal to the hexagonal plane in rod or column form. In one embodiment, the copper-based precipitates measure about 5 nm in diameter and may contain one or more additional alloying elements such as iron, nickel, chromium, cobalt, and/or manganese. These alloying elements may be present only in small amounts. The copper-based precipitates are coherent with the martensite matrix in this embodiment.

In one embodiment, high toughness can be achieved by controlling the nickel content of the matrix to ensure a ductile-to-brittle transition sufficiently below room temperature. The Ductile-to-Brittle Transition Temperature (DBTT) can be decreased by about 16° C. per each weight percent of nickel added to the steel. However, each weight percent of nickel added to the steel can also undesirably decrease the  $M_s$  by about 28° C. Thus, to achieve a DBTT below room temperature while keeping the  $M_s$  above about 50° C., the nickel content in one embodiment is about 6.5 to about 7.5 Ni by weight percent. This embodiment of the alloy shows a ductile-to-brittle transition at about -15° C. The toughness can be further enhanced by a fine dispersion of VN grain-refining particles that are soluble during homogenization and subsequently precipitate during forging.

The alloy may be subjected to various heat treatments to achieve the martensite structure and allow the copper-based precipitates and nitride precipitates to nucleate and grow. Such heat treatments may include hot isostatic pressing, a solutionizing heat treatment, and/or an aging heat treatment. In one embodiment, any heat treatment of the alloy is conducted in a manner that passes through the austenite phase and avoids formation of the ferrite phase. As described above, the ferrite phase has low nitrogen solubility, and can result in undissolved nitrogen escaping the alloy.

Table 1 lists various alloy compositions according to different embodiments of the invention. In various embodiments of the alloy described herein, the material can include a variance in the constituents in the range of plus or minus 5 percent of the stated value, which is signified using the term "about" in describing the composition. Table 1 discloses mean values for each of the listed alloy embodiments, and incorporates a variance of plus or minus 5 percent of each mean value therein. Additionally, an example is described below utilizing the alloy embodiment identified as Steel A in Table 1.

TABLE 1

| wt %    | Fe   | C     | Co  | Cr   | Cu  | Ni  | Mo  | Mn  | N    | Si  | V   | W    |
|---------|------|-------|-----|------|-----|-----|-----|-----|------|-----|-----|------|
| Steel A | Bal. | 0.015 | 3.0 | 11.0 | 0.8 | 7.0 | 1.0 | 0.5 | 0.08 | 0.3 | 0.1 | 0.01 |
| Steel B | Bal. | 0.015 | —   | 12.5 | 1.9 | 2.0 | 0.7 | 0.5 | 0.10 | 0.3 | 0.1 | —    |
| Steel C | Bal. | 0.015 | —   | 11.0 | 2.3 | 2.0 | 0.6 | 0.5 | 0.08 | 0.3 | 0.1 | —    |
| Steel D | Bal. | 0.015 | —   | 12.5 | 1.9 | 3.0 | 1.5 | 0.5 | 0.10 | 0.3 | 0.1 | —    |
| Steel E | Bal. | 0.015 | —   | 11.0 | 0.8 | 6.2 | 1.0 | 0.5 | 0.08 | 0.3 | 0.1 | —    |

## Example 1: Steel A

Steel A was sand cast, and nitrogen-bearing ferro-chrome was added during melt. The casting weighed about 600 pounds. The  $M_s$  for this steel was confirmed as 186°C. using dilatometry. The steel was subjected to a hot isostatic pressing at 1204°C. and 15 ksi Ar for 4 hours, solutionized at 875°C. for 1 hour, quenched with oil, immersed in liquid nitrogen for 2 hours, and warmed in air to room temperature. In the as-solutionized state, the hardness of Steel A was measured at about 36 on the Rockwell C scale. Samples of Steel A were then subjected to an isothermal aging heat treatment at temperatures between 420 and 496°C. for 2 to 32 hours. As shown in FIG. 1, tests performed after the isothermal aging showed that the hardness of the alloy increases rapidly during the isothermal aging process and remains essentially constant at all subsequent times examined. The testing also showed that aging at 482°C. results in a higher impact toughness. Aging the invented steel at 482°C. for 4 hours resulted in a desirable combination of strength and toughness for the alloy evaluated. The tensile yield strength in this condition was about 1040 to 1060 MPa (151 to 154 ksi) and ultimate tensile strength was about 1210 to 1230 MPa (176 to 179 ksi). The ambient impact toughness in this condition was about 19 ft-lb, and the ductile-to-brittle transition was at about -15°C. FIG. 2 shows an atom-probe tomography of this condition where rod-shaped nitride precipitates nucleate on spherical copper-base precipitates.

Variants of the invention facilitate manufacture of case hardened alloy articles which exhibit the superior core characteristics disclosed. The target or design compositions and the actual or measured compositions of five variants of the invention are set forth in Table 2.

casting. The variant alloys thus efficiently enable manufacture of a case hardened component with lower cobalt and nickel content thereby enhancing the opportunity for transformation into a martensitic phase at a reasonable transformation temperature while simultaneously increasing the carbon content to maintain core mechanical properties. The chromium content is increased or maintained for corrosion resistance. The inclusion of a lower cobalt content in combination with copper-nucleated nitride particles results in both surface hardening and superior core mechanical properties. Secondary hardening during tempering is achieved by the simultaneous precipitation of copper-nucleated nitride particles in the nitride case and copper-nucleated carbide particles in the core to provide the combination of surface and core properties. Processability opportunities are also enhanced inasmuch as the alloy may be worked and subsequently case hardened.

TABLE 3

| Core Mechanical Property     | N63-2A<br>(482°C. temper) | N63-2B<br>(482°C. temper) | N63-3A<br>(482°C. temper) | N63-3B<br>(482°C. temper) | N63-3C<br>(482°C. temper) |
|------------------------------|---------------------------|---------------------------|---------------------------|---------------------------|---------------------------|
| Tensile Strength (ksi)       | 223                       | 206                       | 190                       | 198                       | 202                       |
| Tensile Yield Strength (ksi) | 172                       | 163                       | 151                       | 156                       | 155                       |
| % Elongation                 | 23                        | 22                        | 20                        | 20                        | 19                        |
| % Reduction in Area          | 71                        | 73                        | 64                        | 71                        | 59                        |

TABLE 2

| Actual (measured) Chemistry Analysis (wt %) |        |       |       |       |       |      |       |       |       |       |       |         |         |         |         |         |
|---------------------------------------------|--------|-------|-------|-------|-------|------|-------|-------|-------|-------|-------|---------|---------|---------|---------|---------|
| Wt %                                        | C      | Cr    | Ni    | Mo    | Co    | Cu   | Nb    | Ti    | Mn    | Si    | Al    | P       | S       | N       | O       |         |
| N63-2A                                      | Design | 0.14  | 12.5  | 1.5   | 1.5   | 3    | 0.5   | 0.06  | —     | —     | <0.04 | —       | <20 ppm | <20 ppm | <5 ppm  | <60 ppm |
|                                             | Actual | 0.138 | 12.4  | 1.40  | 1.54  | 2.78 | 0.32  | 0.053 | 0.006 | —     | 0.009 | —       | 5 ppm   | 8 ppm   | 23 ppm  | 29 ppm  |
| N63-2B                                      | Design | 0.2   | 12.5  | 1.7   | 1.5   | —    | 0.5   | 0.04  | —     | <0.04 | —     | <20 ppm | <20 ppm | <5 ppm  | <60 ppm |         |
|                                             | Actual | 0.197 | 12.0  | 1.66  | 1.52  | —    | 0.29  | 0.042 | 0.013 | —     | 0.011 | —       | 5 ppm   | 9 ppm   | 14 ppm  | 29 ppm  |
| N63-3A                                      | Design | 0.1   | 12.5  | 1.3   | 1.3   | 3    | 0.5   | 0.05  | 0.01  | —     | —     | <20 ppm | <20 ppm | <10 ppm | <50 ppm |         |
|                                             | Actual | 0.098 | 12.92 | 1.29  | 1.30  | 3.03 | 0.41  | 0.052 | 0.008 | 0.01  | 0.04  | 0.002   | 10 ppm  | 13 ppm  | 10 ppm  | 90 ppm  |
| N63-3B                                      | Design | 0.12  | 13.5  | 1.2   | 0.9   | 3.2  | 0.3   | 0.04  | 0.01  | —     | —     | <20 ppm | <20 ppm | <10 ppm | <50 ppm |         |
|                                             | Actual | 0.121 | 13.88 | 1.18  | 0.874 | 3.01 | 0.327 | 0.051 | 0.015 | 0.01  | 0.007 | 0.002   | 10 ppm  | 15 ppm  | 10 ppm  | 100 ppm |
| N63-3C                                      | Design | 0.15  | 13.5  | 0.4   | —     | 1.7  | 0.3   | 0.04  | 0.01  | —     | —     | <20 ppm | <20 ppm | <10 ppm | <50 ppm |         |
|                                             | Actual | 0.143 | 14.08 | 0.355 | 0.021 | 1.55 | 0.269 | 0.042 | 0.012 | 0.02  | 0.01  | 0.001   | 10 ppm  | 16 ppm  | 10 ppm  | 90 ppm  |
| Intentional alloying elements               |        |       |       |       |       |      |       |       |       |       |       |         |         |         |         |         |
| Impurities/Incidentals                      |        |       |       |       |       |      |       |       |       |       |       |         |         |         |         |         |

A distinction of the constituent range of the variant alloys of Table 2 and the range of constituents associated with the embodiments of the alloys set forth in Table 1 is the following:

Ni: expand to (at least) 0.3-7.5 wt %

Cr: expand to (at least) 10.0-14.5 wt %

Cu: expand to (at least) 0.25-2.3 wt %

C: expand to (at least) up to about 0.2 wt %

V: expand to (at least) up to about 0.15 wt %

Mo: expand to (at least) up to about 0.60-2.0 wt %

Table 3 sets forth mechanical properties associated with each of the five representative alloy variants of Table 2 including the ultimate tensile strength, tensile yield strength, percent elongation and reduction in area due to working and fracture toughness. The compositions of the disclosed embodiments result in a combination of carbon and nitrogen in wt % in the range of about 4-5.5 to 6 in the case of a

TABLE 3-continued

| Core Mechanical Property    | N63-2A<br>(482°C. temper) | N63-2B<br>(482°C. temper) | N63-3A<br>(482°C. temper) | N63-3B<br>(482°C. temper) | N63-3C<br>(482°C. temper) |
|-----------------------------|---------------------------|---------------------------|---------------------------|---------------------------|---------------------------|
| Fracture Toughness (ksi/in) | 60                        | 52                        | 92                        | 79                        | 111                       |

Following are examples of the variant alloys:

## Example 2

Invented steels N632A and N632B were melted as 30 lb. ingots using vacuum induction melting (VIM), and secondary melted using vacuum arc remelting (VAR). In contrast to the alloy variant of EXAMPLE 1, this variant is not melted

with deliberate additions of nitrogen. Melted ingots were processed by conventional means, including homogenization in the range of 1100° C. to 1200° C. and hot rolling from a starting temperature in the range of 1100° C. to 1200° C. to form the material into plate. To introduce nitrogen into a case hardened layer, samples were nitrided at 1100° C. for about 4 hours using a low-pressure solution nitriding process, followed by gas quenching to room temperature and subsequent cryogenic treatment for martensitic transformation. Samples were subjected to an isothermal aging treatment at temperatures in the range of 420° C. to 496° C. for up to 32 hours, resulting in simultaneous precipitation of copper-nucleated nitride particles in the case layer and copper-nucleated carbide particles in the core material. Testing indicated a desirable combination of case and core properties when the invented steel was aged at 482° C. for 8 hours. As set forth in Table 3, the tensile yield strength in this condition was about 1124 to 1186 MPa (163 to 172 ksi), and the ultimate tensile strength was about 1420 to 1538 MPa (206 to 223 ksi). The ambient temperature fracture toughness (measured according to ASTM E399 standards) in this condition was about 57 to 66 MPa·m<sup>0.5</sup> (52 to 60 ksi·in). As set forth in FIG. 3, the demonstrated case hardness in this condition was about 59 to 61 on the Rockwell C scale.

Thus, the alloy variants of Table 2 are designed to be case hardenable. The alloys as described and processed with respect with Table 1 are deliberately alloyed with nitrogen during the melting process to yield a specific Carbon+Nitrogen (C+N) content to achieve a microstructure (Copper-nucleated  $M_2N$  precipitation within a martensitic stainless steel) that yields specific novel properties. The variants of Table 2 alloys utilize essentially the same microstructural approach or concept (Copper-nucleated  $M_2N$  precipitation within a martensitic stainless steel including the feature of matrix) to achieving high surface hardness in a case-hardenable alloy, but with no deliberate nitrogen during melting. Modifications to the variant alloy design to achieve this include:

Equivalent C+N alloying content is maintained during melting, but C is favored for conventional melt processing and core mechanical properties

High nitrogen contents necessary for case hardness are incorporated using a secondary processing step of "Solution Nitriding". Solution nitriding results in ~0.3 wt % N in the case, maintaining a N/C ratio consistent with the alloys of Table 1.

High surface hardness is achieved through Copper-nucleated  $M_2N$  precipitation in the case during tempering

High nitrogen content in the case lowers the martensite transformation temperature, and so nickel content is lowered to raise the Ms temperature of the case an acceptable level to avoid retained austenite phase (austenite being detrimental to surface hardness and  $M_2N$  precipitation)

A graphical description of the processing used to create the case hardened alloys such as set forth in Table 2 vis a vis the alloy form represented by the examples in Table 1 is set forth in FIG. 6.

In addition to the enhanced physical characteristics of the case and the maintenance of desirable mechanical and physical characteristics of the core, the alloys of the invention have high corrosion resistance as exemplified by FIG. 5 using a standard salt fog test wherein the alloys were exposed to hostile environments in contrast to control alloys 440C manufactured by in contrast to control alloy 440C manufactured at Latrobe Specialty Steel by double vacuum melting and in accordance with Aerospace Material Speci-

fication (AMS) 5630. The test results demonstrate the significantly improved corrosion resistance associated with the variant alloys described.

Microstructure analysis of the alloys results in a case hardened martensitic phase comprising at least about 90% by volume and typically in the range of 95% to 100% with a case thickness dependent upon the conditions of the nitriding process (in the range of 0.5 mm to 2 mm in the embodiments disclosed here).

The various embodiments of martensitic stainless steels disclosed herein provide benefits and advantages over existing steels, including existing secondary-hardened carbon stainless steels or conventional nitride-strengthened steels. For example, the disclosed steels provide a substantially increased strength and avoid embrittlement under impact loading, at attractively low material and process costs. Additionally, cementite formation in the alloy is minimized or substantially eliminated, which avoids undesirable properties that can be created by cementite formation. Accordingly, the disclosed stainless steels may be suitable for gear wheels where high strength and toughness are desirable to improve power transmission. Other benefits and advantages are readily recognizable to those skilled in the art.

Several alternative embodiments and examples have been described and illustrated herein. A person of ordinary skill in the art would appreciate the features of the individual embodiments, and the possible combinations and variations of the components. A person of ordinary skill in the art would further appreciate that any of the embodiments could be provided in any combination with the other embodiments disclosed herein. "Providing" an alloy, as used herein, refers broadly to making the alloy, or a sample thereof, available or accessible for future actions to be performed thereon, and does not connote that the party providing the alloy has manufactured, produced, or supplied the alloy or that the party providing the alloy has ownership or control of the alloy. It is further understood that the invention may be in other specific forms without departing from the spirit or central characteristics thereof. The present examples therefore are to be considered in all respects as illustrative and not restrictive, and the invention is not to be limited to the details given herein. Accordingly, while the specific examples have been illustrated and described, numerous modifications come to mind without significantly departing from the spirit of the invention and the scope of protection is only limited by the scope of the accompanying claims.

#### What is claimed is:

1. A method of manufacture of case hardened martensitic stainless steel alloy strengthened by copper-nucleated nitride precipitates, said alloy comprising, in combination elemental constituents by weight percent, about 10.0 to about 14.5 Cr, about 0.3 to about 7.5 Ni, up to about 17.0 Co, about 0.6 to about 1.5 Mo, about 0.25 to about 2.3 Cu, up to about 0.6 Mn, up to about 0.4 Si, about 0.05 to about 0.15 V, up to about 0.10 N, up to about 0.2 C, up to about 0.01 W, and the balance Fe and incidental elements and impurities, said alloy having a microstructure substantially free of cementite carbides and comprising a martensite matrix with nanoscale copper particles and alloy nitride precipitates selected from the group consisting of alloy nitride precipitates enriched with a transition metal nucleated on the copper precipitates, said alloy nitride precipitates having a hexagonal structure, said alloy nitride precipitates including one or more alloying elements selected from the group Fe, Ni, Cr, Co and Mn coherent with the matrix, and said alloy nitride precipitates having two dimensional coherency with the matrix, said

alloy substantially free of cementite carbide precipitates in the form of a case hardened article of manufacture, comprising the steps of:

formulating a melt  
preparing a melt in accord with the elemental constituents; 5  
casting the melt in a form;  
homogenizing said form; and  
aging the form.

2. The process of claim 1 absent the inclusion of an 10  
elemental constituent of N in the melt, and aging in combination with solution treatment with N.

3. The method of claim 1 in combination with a predicate 15  
step of the forging or hot isostatic pressing in combination  
with aging.

4. The method of claim 2 in combination with a predicate  
step of forging or hot isostatic pressing in combination with 20  
aging.

5. The method of claim 1 in combination with a terminal  
step of forging. 25

6. The method of claim 2 in combination with a terminal  
step of forging.

7. The method of claim 3 in combination with a terminal  
step of forging.

8. The method of claim 4 in combination with a terminal 25  
step of forging.

\* \* \* \* \*